

June 19, 1956

G. M. HOOD ET AL

2,751,297

PHOTOGRAPHIC EMULSION LAYER CONTAINING A 3-PYRAZOLIDONE

Filed Aug. 3, 1953



GLAY M. HOOD  
PAUL R. CROOKSHANK  
INVENTORS

BY *Daniel L. Mayne*  
*W. H. McJowell*  
ATTORNEY & AGENT

1

2,751,297

## PHOTOGRAPHIC EMULSION LAYER CONTAINING A 3-PYRAZOLIDONE

Glenn M. Hood and Paul R. Crookshank, Rochester, N. Y., assignors to Eastman Kodak Company, Rochester, N. Y., a corporation of New Jersey

Application August 3, 1953, Serial No. 371,948

12 Claims. (Cl. 95—7)

This invention relates to photographic emulsions and particularly to photographic emulsions containing 3-pyrazolidone compounds as development accelerating and emulsion stabilizing agents.

In the development of many types of photographic emulsion layers, particularly in the case of washed silver bromide emulsion layers used on sensitive paper products, it is desirable to obtain rapid and reasonably complete development of the exposed emulsion layer. We have discovered that if certain 3-pyrazolidone compounds are incorporated into silver halide emulsion layers, particularly those emulsion layers which are normally slow developing or in those cases where a short complete development is desired, development proceeds much faster than when the 3-pyrazolidone compounds are not present in the emulsion layer.

The accompanying drawings show in greatly enlarged cross-sectional view the appearance of a representative photographic element contemplated by our invention. In the element of the drawings layer 10 represents a support such as paper, cellulose ester, etc., and layer 11 the emulsion layer of the invention containing a mixture of silver halide and a 3-pyrazolidone compound.

The 3-pyrazolidone compounds employed in the emulsions have the general structure



in which the various R groups represent substituents such as hydrogen, alkyl heterocyclic or aryl groups, for example, R can be benzothiazolyl or an aryl group of the benzene or naphthalene series, substituted or not; however, R cannot be a hydrogen atom inasmuch as 3-pyrazolidone compounds containing no substituent other than hydrogen in the 1-position of the nucleus, such as 3-pyrazolidone itself, are not effective in our invention. R<sub>1</sub>, R<sub>2</sub>, R<sub>3</sub> and R<sub>4</sub> can be hydrogen atoms or alkyl groups preferably containing from 1 to 4 carbon atoms, or aryl groups such as phenyl and naphthyl, substituted or not.

The compounds are not to be confused with 5-pyrazolidones such as 1-phenyl-5-pyrazolidone.

The following compounds are representative of the 3-pyrazolidone compounds useful in emulsions for the purposes of our invention.

1. 1-phenyl-3-pyrazolidone
2. 1-p-tolyl-3-pyrazolidone
3. 5-phenyl-3-pyrazolidone
4. 5-methyl-3-pyrazolidone
5. 1-p-chlorophenyl-3-pyrazolidone
6. 1-phenyl-5-phenyl-3-pyrazolidone
7. 1-m-tolyl-3-pyrazolidone
8. 1-phenyl-5-methyl-3-pyrazolidone
9. 1-p-tolyl-5-phenyl-3-pyrazolidone
10. 1-m-tolyl-3-pyrazolidone

2

11. 1-p-methoxyphenyl-3-pyrazolidone
12. 1-acetamidophenyl-3-pyrazolidone
13. 1-phenyl-2-acetyl-4,4-dimethyl-3-pyrazolidone
14. 1-phenyl-4,4-dimethyl-3-pyrazolidone
15. 1-m-aminophenyl-4-methyl-4-propyl-3-pyrazolidone
16. 1-o-chlorophenyl-4-methyl-4-ethyl-3-pyrazolidone
17. 1-m-acetamidophenyl-4,4-diethyl-3-pyrazolidone
18. 1-(p-β-hydroxyethylphenyl)-4,4-dimethyl-3-pyrazolidone
19. 1-p-hydroxyphenyl-4,4-dimethyl-3-pyrazolidone
20. 1-p-methoxyphenyl-4,4-diethyl-3-pyrazolidone
21. 1-p-tolyl-4,4-dimethyl-3-pyrazolidone
22. 1-(7-hydroxy-2-naphthyl)-4-methyl-4-n-propyl-3-pyrazolidone
23. 1-p-diphenyl-4,4-dimethyl-3-pyrazolidone
24. 1-(p-β-hydroxyethylphenyl)-3-pyrazolidone
25. 1-o-tolyl-3-pyrazolidone
26. 1-o-tolyl-4,4-dimethyl-3-pyrazolidone
27. 1-benzothiazolyl-3-pyrazolidone

Compounds 1 to 12 can be prepared by the methods described in British Patents 679,677 and 679,678. Compounds 13 to 23 and 26 above are representative of 4,4-dialkyl-3-pyrazolidone compounds useful in the invention and these compounds are described and claimed in the Allen et al. U. S. patent application Serial No. 372,148, filed August 3, 1953.

The  $\omega$ -hydroxyalkylphenyl-3-pyrazolidones in which the alkyl group preferably contains from 1 to 4 carbon atoms, for example, compounds 18 and 24 above, are described in the Allen et al. invention and in the Reynolds and Tinker U. S. patent application Serial No. 372,167, filed concurrently.

The 3-pyrazolidone compounds can be used in silver halide emulsions for the purposes of the invention with gratifying results in a rather wide range of concentration. Useful results can be obtained, for example, with from about 0.2 to 2.0 grams of the 3-pyrazolidone compound per mol of silver nitrate used in making the emulsion and converted to silver halide. However, both smaller and larger quantities of the compounds than indicated can be used with good results. The particular silver halide in the emulsion is not especially critical nor is the particular method used for preparing the emulsion. Thus one or more of the 3-pyrazolidone compounds can be added to emulsions containing mixtures of silver bromide, silver chloride and silver iodide such as present in emulsion of well known types. However, the 3-pyrazolidones are particularly useful in conjunction with bromoiodide emulsions which normally develop slowly and in emulsions which normally require a short first development as in bleach redevelopment reversal processes. The 3-pyrazolidone compounds are added in water solution to the emulsions at any stage in their preparation but are conveniently added after the final digestion and just before coating.

As will be apparent, the emulsions may contain the usual addenda including antifoggants, spreading agents, coupler compounds, etc. Such emulsions are adaptable to use in forming single as well as multi-layer films useful in color photography which customarily include two or more emulsion layers on a support sensitized to different regions of the visible spectrum and which may or may not contain coupler compounds. According to our invention, such color films carry at least one emulsion layer containing one or more of the pyrazolidone compounds of the invention.

If desired, a portion or all of the 3-pyrazolidone compound required to accelerate the development of the emulsion or to stabilize it can be incorporated in a hydrophilic colloid layer such as gelatin adjacent to the emulsion layer with the result that material development acceleration and improvement in emulsion stability are obtained thereby.

The hydrophilic colloid vehicle of the emulsions containing the 3-pyrazolidone compounds can be, for example, gelatin, polyvinyl alcohol, partially hydrolyzed cellulose esters and copolymers of polyvinyl alcohol and the like.

## EXAMPLE 1

Samples of a finished washed bromo-iodide emulsion were provided. To the respective samples of melted emulsion were added aqueous solutions of the 3-pyrazolidone compounds indicated in the following table. The samples were coated successively on a paper stock and dried. The samples were then given continuous wedge exposures and developed for 20 to 45 seconds both when the samples were fresh and after 3-day incubation at 120° F. and 60 percent relative humidity, development being carried out in a conventional Elon-hydroquinone developer. Sensitometric evaluation of the developed samples produced the data tabulated in the following table. The "bar gamma" values in the table are a measure of the contrast of the developed samples and a description of the determination of this value is given in the American Standards Association Bulletin entitled "Sensitometry and Grading of Photographic Papers," January 8, 1953. In considering the data of the table, the development acceleration effect of using the 3-pyrazolidone compounds in the emulsions should be made between samples developed for 20 seconds and the stabilizing effect of the compounds should be evaluated on the basis of the samples developed for 45 seconds. It will be apparent from the data that the 3-pyrazolidone compounds materially increase the contrast of the emulsion and stabilize the emulsion against contrast loss on aging.

## Use of pyrazolidones in a washed bromoiodide emulsion

| Chemical                                                 | Concen-<br>tration,<br>mg./mole<br>Silver<br>Halide | Bar Gamma    |               |              |               | D-max.       |               |              |               |
|----------------------------------------------------------|-----------------------------------------------------|--------------|---------------|--------------|---------------|--------------|---------------|--------------|---------------|
|                                                          |                                                     | 20 Sec. Dev. |               | 45 Sec. Dev. |               | 20 Sec. Dev. |               | 45 Sec. Dev. |               |
|                                                          |                                                     | Fresh        | 3 Day<br>Inc. | Fresh        | 3 Day<br>Inc. | Fresh        | 3 Day<br>Inc. | Fresh        | 3 Day<br>Inc. |
| Check.....                                               | None                                                | 1.00         | .81           | 1.72         | 1.50          | 1.01         | .89           | 1.26         | 1.25          |
|                                                          | 1,750                                               | 1.68         | 1.35          | 1.85         | 1.85          | 1.26         | 1.19          | 1.26         | 1.30          |
| 1-phenyl-3-pyrazolidone.....                             | 875                                                 | 1.50         | 1.07          | 1.94         | 1.71          | 1.16         | 1.14          | 1.26         | 1.28          |
|                                                          | 437                                                 | 1.41         | .95           | 1.86         | 1.70          | 1.16         | 1.12          | 1.27         | 1.28          |
|                                                          | 219                                                 | 1.21         | .93           | 1.89         | 1.66          | 1.15         | 1.04          | 1.27         | 1.26          |
|                                                          | 1,750                                               | 1.31         | 1.13          | 1.81         | 1.79          | 1.21         | 1.13          | 1.28         | 1.30          |
| 4,4-dimethyl-1-phenyl-3-pyrazolidone.....                | 875                                                 | 1.37         | 1.09          | 1.82         | 1.74          | 1.19         | 1.08          | 1.27         | 1.28          |
|                                                          | 437                                                 | 1.25         | .98           | 1.85         | 1.65          | 1.15         | 1.10          | 1.27         | 1.27          |
|                                                          | 219                                                 | 1.20         | .93           | 1.83         | 1.65          | 1.15         | 1.00          | 1.27         | 1.28          |
| 4,4-dimethyl-1-(p-tolyl)-3-pyrazolidone.....             | 1,750                                               | 1.51         | 1.16          | 1.75         | 1.77          | 1.23         | 1.02          | 1.28         | 1.28          |
|                                                          | 875                                                 | 1.45         | 1.00          | 1.75         | 1.67          | 1.17         | 1.10          | 1.27         | 1.28          |
|                                                          | 437                                                 | 1.29         | .96           | 1.61         | 1.62          | 1.10         | 1.05          | 1.23         | 1.26          |
|                                                          | 219                                                 | .76          | .96           | 1.71         | 1.64          | .98          | 1.02          | 1.25         | 1.24          |
| 1-(4- <i>p</i> -Hydroxyethyl-phenyl)-3-pyrazolidone..... | 1,750                                               | 1.72         | 1.06          | 1.80         | 1.69          | 1.13         | 1.12          | 1.27         | 1.27          |
|                                                          | 875                                                 | 1.61         | .95           | 1.74         | 1.67          | 1.10         | 1.07          | 1.26         | 1.26          |
|                                                          | 437                                                 | 1.65         | .91           | 1.71         | 1.62          | 1.06         | 1.03          | 1.26         | 1.26          |
|                                                          | 219                                                 | 1.59         | .80           | 1.69         | 1.55          | 1.04         | 1.10          | 1.25         | 1.24          |

## EXAMPLE 2

To a sample of a normally slow-developing bromo-iodide emulsion used in reversal processes was added 8.77 milligrams of 1-phenyl-3-pyrazolidone per mol of silver nitrate used in making the emulsion and converted to silver halide. The emulsion was coated as usual on a paper base, exposed, developed in a caustic hydroquinone developer and evaluated sensitometrically. The data obtained showed that the gamma for samples of the emulsion containing no pyrazolidone compound which were developed 15, 30 and 45 seconds respectively, were 0.75, 0.98 and 1.05, whereas the samples containing the pyrazolidone compound developed under the same conditions had gammas of 1.08, 1.27 and 1.35. This example illustrates the effect which may be expected in reversal processes where it is desired to obtain a rapid complete development of the negative image where the first or negative development is usually short.

The other 3-pyrazolidone compounds such as those specifically mentioned above are useful in our invention as accelerators and stabilizers for emulsions. As men-

tioned previously, it appears essential that the 3-pyrazolidone compounds contain a substituent other than hydrogen in the 1-position of the nucleus since compounds such as 3-pyrazolidone do not produce the desired effect when incorporated into silver halide emulsion layers.

What we claim is:

1. A light-sensitive photographic emulsion comprising a mixture of unexposed silver halide and a 3-pyrazolidone having the following general structure



wherein R represents a member of the group consisting of heterocyclic groups and aryl groups of the benzene and naphthalene series and R<sub>1</sub>, R<sub>2</sub>, R<sub>3</sub> and R<sub>4</sub> each represent a member of the group consisting of a hydrogen atom, a mononuclear aryl group of the benzene series, and an alkyl group containing from 1 to 4 carbon atoms, in a small amount not in excess of about 2 grams per mol of silver halide in the emulsion.

2. A light-sensitive photographic emulsion comprising a mixture of unexposed silver halide and a 3-pyrazolidone having the following general structure



30

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

## 5

ing a mixture of unexposed silver halide and a 3-pyrazolidone having the following general structure



wherein R represents a mononuclear aryl group of the benzene series, in a small amount not in excess of about 2 grams per mol of silver halide in the emulsion.

7. A light-sensitive photographic emulsion layer comprising a mixture of unexposed silver halide and 1-phenyl-3-pyrazolidone, in a small amount not in excess of about 2 grams per mol of silver halide in the emulsion.

8. A light-sensitive photographic emulsion layer comprising a mixture of unexposed silver halide and a 1-tolyl-3-pyrazolidone, in a small amount not in excess of about 2 grams per mol of silver halide in the emulsion.

9. A light-sensitive photographic emulsion layer comprising a mixture of unexposed silver halide and 1-p-tolyl-3-pyrazolidine, in a small amount not in excess of about 2 grams per mol of silver halide in the emulsion.

10. A light-sensitive photographic emulsion layer comprising a mixture of unexposed silver halide and a 1- $\omega$ -hydroxyalkylphenyl-3-pyrazolidone, in a small amount not in excess of about 2 grams per mol of silver halide in the emulsion.

11. A light-sensitive photographic emulsion layer comprising a mixture of unexposed silver halide and 1-(p- $\beta$ -hydroxy-ethylphenyl)-3-pyrazolidone, in a small amount not in excess of about 2 grams per mol of silver halide in the emulsion.

10

15

20

25

30

## 6

12. A light-sensitive photographic element comprising a support, an unexposed silver halide emulsion layer, and a hydrophilic colloid layer adjacent to said emulsion layer containing a 3-pyrazolidone having the following general structure



wherein R represents a member of the group consisting of heterocyclic groups and aryl groups of the benzene and naphthalene series and R<sub>1</sub>, R<sub>2</sub>, R<sub>3</sub> and R<sub>4</sub> each represent a member of the group consisting of a hydrogen atom, a mononuclear aryl group of the benzene series, and an alkyl group containing from 1 to 4 carbon atoms, in a small amount not in excess of about 2 grams per mol of silver halide in the emulsion.

## References Cited in the file of this patent

## UNITED STATES PATENTS

|           |                   |               |
|-----------|-------------------|---------------|
| 742,405   | Eichengrun et al. | Oct. 27, 1903 |
| 2,477,462 | McQueen           | July 26, 1949 |
| 2,672,416 | Stanton           | Mar. 16, 1954 |

## FOREIGN PATENTS

|         |               |                |
|---------|---------------|----------------|
| 679,677 | Great Britain | Sept. 24, 1952 |
| 679,678 | Great Britain | Sept. 24, 1952 |